

3,510,282  
NAPHTHENYL-ACYLATED POLYAMINES  
AND USES

William E. Seffens, St. Louis, Mo., assignor to Petrolite Corporation, Wilmington, Del., a corporation of Delaware  
No Drawing. Filed Aug. 11, 1967, Ser. No. 659,875  
Int. Cl. C10I 1/22, 1/18

U.S. CL. 44—63

1 Claim

### ABSTRACT OF THE DISCLOSURE

Acylated polyamines such as compounds of the formulae:

(1)



(3) salts of (1) and (2), and (4) mixtures of (1) and (2) and/or (3); where R is a naphthyl moiety, A and A' are alkylene moieties (straight chain or branched), and X is a polar moiety such as, for example, hydroxy, amino, carboxyl-containing, etc.; and to hydrocarbon fuels in the gasoline range containing said compounds. These fuels possess anti-icing, anti-fouling and corrosion inhibiting properties.

This invention relates to acylated polyamines such as compounds of the formulae:

(1)



(3) salts of (1) and (2), and (4) mixtures of (1) and (2) and/or (3); where R is a naphthyl moiety, A and A' are alkylene moieties (straight chain or branched), and X is a polar moiety such as, for example, hydroxy, amino, carboxyl-containing, etc.; and to hydrocarbon fuels in the gasoline range containing said compounds. These fuels possess anti-icing, anti-fouling and corrosion inhibiting properties.

### THE ICING PROBLEM

Engine stalling due to carburetor icing occurs most frequently under engine idling conditions and particularly under weather conditions of relatively high humidity and at a temperature below about 60° F. While this problem has been in existence for many years, it has of late become of increased importance because of recent engine design. Most post-war cars are provided with automatic chokes and provide no means for manual operation of the throttle so that operators of such cars are no longer able to regulate idle speeds during warm-up periods to prevent stalling. Furthermore, the idle speed of automobiles equipped with automatic transmissions is rather critical during the warm-up period and the fastest idle rate which may be used is limited to avoid creeping. Another factor in carburetor icing is the high volatility of motor fuels now provided for present-day engines.

It has been established that the cause of engine stalling in cool humid weather is the formation of ice in the engine carburetor. On such cool moist days, the gasoline evaporated in the carburetor produces a sufficient refrigerating effect to condense and freeze the moisture present in the air entering the carburetor. Fuel vaporization in the fuel carburetor under such conditions can cause a temperature drop in the carburetor of up to 50° F.

below that of the entering air; as a result, up to the time of complete engine and radiator warm-up, this drop in temperature causes formation of ice crystals in the carburetor. The maximum refrigeration of the type referred to takes place under conditions of light load operation. As cooling of the carburetor parts takes place, ice begins to form as soon as these parts are refrigerated to a temperature below about 30° F., so that, when the throttle is closed to the idle position, the ice formed in the carburetor, particularly that formed on the throttle plate and the adjacent walls, closes the narrow air ports, thereby restricting the normal flow of the air to the engine, causing repeated engine stalling. While an engine stalled, because of carburetor icing, can be readily started because the ice formed melts almost immediately due to residual heat from the exhaust manifold, it is highly desired to avoid any stalling due to carburetor icing because of the attendant inconvenience. For example, stalling due to carburetor icing of a car, equipped with automatic transmission, frequently does not occur until the driver is ready to accelerate so that at this most inconvenient time it is necessary to shift the car to neutral, restart the engine and shift back into gear, all of which magnifies the inconvenience of frequent stalls.

25 In addition, it is well known that commercial gasolines themselves contain small amounts of dissolved water. Some additional moisture tends to accumulate in the fuel tanks of cars, hence water is always present in the fuel passing through the engine's fuel supply system. When exposed to temperatures below 32° F., and particularly at temperatures below 20° F., the water content of a fuel freezes and tends to form ice crystals in the supply system. These ice crystals can restrict and even block the small diameter fuel line or the small openings present 30 in the fuel filter, thus impairing and ultimately disrupting engine operation.

### THE FOULING PROBLEM

In the course of operation of an internal combustion engine, deposits build up in the throat of a carburetor, particularly in the area adjacent to the throttle plate. These deposits have a choking effect on the engine, thereby causing rough idling, and in many cases, the occurrence of frequent stalling.

45 It is generally accepted theory that these deposits form from solid particulate matter borne by the copious quantities of intake air an operating carburetor breathes. This solid matter is fed to the air by industrial stacks, and by exhaust pipes and crankcase breathers of motor vehicles, and other sources of fumes and smoke. It is, therefore, desirable to provide novel fuels which are effective in preventing deposits from forming in the carburetor of an internal combustion engine. The agents so employed are also known as carburetor detergents.

### THE CORROSION PROBLEM

Since water is almost invariably present in the bottom of gasoline storage facilities, the possibilities of rusting and rust contamination of the fuel are excellent, and these are matters of great concern. The sloshing of fuel in storage tanks can slough rust scale off the tank walls, leading to the suspension of rust particles in the fuel itself. The larger of these particles can clog fuel filters, while smaller particles can wend their way into the combustion chambers of an engine and score cylinder walls and valves. The inhibition of rusting is therefore an important desideratum, and one which can be realized by using the novel fuels of this invention.

I have now prepared novel compositions comprising 70 naphthenic acid-acylated cyclic amidine-forming polyamines having hydroxy, amino, carboxyl-containing, or other polar groups on the N-bonded side chain. These

compositions are amides, cyclic amidines, salts, and mixtures thereof.

I have also found that hydrocarbons of the gasoline boiling range containing these compositions are multi-functional additives which possess anti-icing, anti-fouling, and corrosion inhibiting properties, as well as other properties.

The cyclic amidines and amides of this invention are prepared by well known methods amply described in the literature. In essence, the preparation involves reacting the naphthenic acid with the polyamine with the elimination of water. Where only one mole of water is removed the amide is formed.



which can be further reacted with the removal of a second mole of water to yield the cyclic amidine, i.e., the imidazoline or tetrahydropyrimidine



The product used may be either the amide, the cyclic amidine or mixtures thereof.

The polyamine reacted is of the formula



where A and A' which need not be the same are for example



etc., and X is for example



where R' is for example a hydrocarbon group, i.e. alkyl, aryl, cycloalkyl, etc., and M is a salt moiety. In the preferred embodiment X is  $-\text{OH}$ .

In certain instances where A is cyclic amidine-forming, A' need not necessarily be cyclic amidine-forming.

In addition the  $-\text{A}'\text{OH}$  side chain may be oxyalkylated to yield with alkylene oxides such as ethylene oxide, propylene oxide, butylene oxide, styrene oxide, or more than one type of oxide to yield  $-(\text{A}'\text{O})_n\text{H}$  units where  $n$  is a whole number such as 1, 2, 3, 4, 5, etc.

Naphthenic acids are employed in the present invention. As to the description of naphthenic acids reference is made to Industrial & Engineering Chemistry, vol. 41, No. 10, October 1949, pp. 2080-2090, as follows:

"The most widely used is naphthenic acid, a petroleum refining by-product obtained when the alkali liquor from the caustic treatment of gas oil is acidified with sulfuric acid. This treatment produces a dark brown about 12 on the Gardner color scale (when cut 1 to 9 with mineral spirits) oily liquid which separates to the top of the aqueous liquor. The mixed acids can be divided roughly into three groups having the general formulas:  $\text{C}_n\text{H}_{2n-2}\text{O}_2$ ,  $\text{C}_n\text{H}_{2n-2}\text{O}_2$ , and  $\text{C}_n\text{H}_{2n-4}\text{O}_2$ . The first group occurs largely in the lower boiling fraction of the mixture. They usually contain 6 or 7 carbon atoms and are colorless. The sec-

ond group, usually the largest, contains acids of 8 to 12 carbon atoms having the structure:



The third group contains the heaviest molecules which are polycyclic and have from 12 to 23 carbon atoms. All 10 fractions from a carefully distilled naphthenic acid (24) contain some color which, so far, has proved impossible to remove. Tarry residues account for the dark color of the crude, but these are largely removed by distillation. Since naphthenic acids are saturated and primarily cyclic, 15 their soaps have much greater stability than those of other common liquid acids. The crude acid as delivered has a density of 8.04 to 8.44 pounds per gallon and a viscosity of 1.25 poises at 77° F. The acid values range from 160 to 270, but naphthenic acid used for soap manufacture usually has an acid value between 220 and 230. 20 pH of the water extract is about 5.5 and the iodine value between 8 and 11. Unsaponifiables are held below 12%. The initial boiling points vary widely from shipment to shipment. Individual batches have boiled below 200° F. 25 and up to almost 400° F. at 3.5 inches of mercury."

A typical formula in connection with some of the commercially available naphthenic acids is the following:



35 These particular acids are available in at least three different grades; Grade 1 having an average molecular weight of 290-300. Generally speaking, there is present about 6% of non-saponifiables and this type is perhaps characteristic of the most common commercially available naphthenic acid.

40 Grade 2 has a somewhat higher molecular weight, for instance 320-330 and contains about 8% of non-saponifiable matter. Grade 3, which finds considerable utility, has a molecular weight range of 410-420 and contains about 10% nonsaponifiable matter.

45 Any naphthenic acid may be used but preference is to use the commercial grades above described, or in some instances, mixtures of two different grades so as to give, for example, an average molecular weight of 360 to 370 in some instance, and in others, a molecular weight of 50 about 310, or thereabouts.

50 In examining the formula immediately preceding, with the formula preceding the above formula, and ignoring difference in the cyclic structure of the naphthenic acids, it is apparent that in at least some naphthenic acids which are available commercially the cyclic structure is part of the beta carbon atom. On the other hand, as far as is known, and referring to the formula



60 there are available naphthenic acids in which apparently  $x$  in the formula represents a small whole number, for instance, 3 or 4 or the like.

65 In practicing the present invention preference is given to the higher molecular weight naphthenic acids, for example those having an average molecular weight of at least about 2000, such as about 250 to 500, or greater, for

example from about 290 to 420 but preferably from about 325-375.

Since commercial grades of naphthenic acids are employed, these contain many individual species over a molecular weight range.

The most preferred naphthenic acid those known as "Sunaptic" acids which are high-molecular-weight naphthenic acids prepared by the caustic extraction of selected base stocks. They range in acid number from 120 to 180, in molecular weight from 300 to 415, and are available in three grades, A, B, and C.

Specifications and typical analyses for the three Sunaptic acids are given in the table below. They are mono-carboxylic acids and, having no olefinic unsaturation, are highly resistant to oxidative rancidity. They have low pour points and contain relatively low amounts of unsaponifiable matter. Sunaptic acids are soluble in most hydrocarbons.

## SPECIFICATIONS

|                                              | Sunaptic Acids A   |                     |                    | Sunaptic Acids B    |                    |                     |
|----------------------------------------------|--------------------|---------------------|--------------------|---------------------|--------------------|---------------------|
|                                              | Specifi-<br>cation | Typical<br>Analysis | Specifi-<br>cation | Typical<br>Analysis | Specifi-<br>cation | Typical<br>Analysis |
| Acid number, mg. KOH/g.                      | 170-180            | 172                 | 150-160            | 157                 | 120-130            | 12                  |
| Unsaponifiables, percent by wt. <sup>1</sup> | 7 max.             | 6.3                 | 7 max.             | 5.0                 | 11 max.            | 9.1                 |
| Density, 20/4                                | 0.987              | 0.987               | 0.987              | 0.987               | 0.987              | 0.987               |
| Specific gravity at 60° F.                   | 0.9902             | 0.9902              | 0.9909             | 0.9909              | 0.9930             | 0.9930              |
| API gravity at 60° F.                        | 11-13              | 11-13               | 11-13              | 10-12               | 11-12              | 11.0                |
| Viscosity, SUS at 210° F.                    | 100-120            | 113                 | 150-200            | 159                 | 350-650            | 430                 |
| Bromine number <sup>2</sup>                  | 9.0                | 9.0                 | 10.0               | 10.0                | 12.1               | 12.1                |
| Refractive index, $n_{D}^{20}$               | 1.498              | 1.498               | 1.507              | 1.507               | 1.516              | 1.516               |
| Pour point, deg F.                           | +30                | +30                 | +45                | +45                 | +75                | +75                 |
| Flash point, deg F.                          | 335 min.           | 330                 | 370 min.           | 445                 | 425 min.           | 445                 |
| Sulfur content, percent by weight            | 0.4 max.           | 0.4 max.            | 0.4 max.           | 0.4 max.            | 0.4 max.           | 0.4 max.            |
| Average molecular weight <sup>3</sup>        |                    | 310                 |                    | 340                 |                    | 415                 |
| Distillation Range, deg F. at 2 mm. Hg:      |                    |                     |                    |                     |                    |                     |
| Initial                                      | 326                |                     | 336                |                     | 408                |                     |
| 5%                                           | 336                |                     | 354                |                     | 427                |                     |
| 10%                                          | 346                |                     | 370                |                     | 446                |                     |
| 50%                                          | 378                |                     | 423                |                     | 509                |                     |
| 90%                                          | 452                |                     | 490                |                     | 580                |                     |
| 95%                                          | 470                |                     | 516                |                     |                    |                     |
| End Point                                    | 486                |                     | 526                |                     | 596                |                     |
| Percent Recovery                             | 98                 |                     | 98                 |                     | 95                 |                     |

<sup>1</sup> A.O.C.S. C-6a-40<sup>2</sup> ASTM D-1158-52T<sup>3</sup> Calculated from Acid Number and Percent Unsaponifiable.

The following example is presented for purposes of illustration and not of limitation.

## EXAMPLE 1

Equimolar amounts of a commercial naphthenic acid, Sunaptic Acid B, (1 mole, 365 parts by weight) and aminoethylethanolamine (1 mole, 104 parts by weight) were charged to a reactor and heated to 170° C. for 30 minutes at which time a vacuum of about 28 inches was applied for an additional 3.5 hours. The product which was predominantly the imidazoline,



with a small amount of amide,



after cooling was dissolved in a hydrocarbon solvent to yield a solution which was 75% active.

The additive used in this invention may be dissolved directly in gasoline. As an alternative procedure a liquid concentrate of the additive may be prepared using as a solvent a hydrocarbon which is either compatible with, or a conventional component of, gasoline compositions. Suitable solvents include toluene, catalytic reformate, neutral oil and the like. The liquid concentrate may then be added to gasoline.

Gasoline base stocks which may be used in the practice of this invention include any of those conventionally used in preparing a motor fuel for a spark-ignited inter-

nal combustion engine, such as catalytic distillate, motor polymer, alkylate, catalytic reformate, isomerate, naphthas, etc. The gasoline will preferably contain an anti-knock agent of the tetra-alkyl lead type, such as tetraethyl lead, tetramethyl lead or chemical or physical mixtures thereof, and a scavenger agent such as ethylene dichloride and/or ethylene dibromide. The amount of anti-knock agent will usually be at a level of approximately 3 ml./gal., but may range from 1/2 ml./gal. to 6 ml./gal. The gasoline may also include other conventional additives such as solvent oils, dyes and the like.

These additives are employed in any suitable concentration capable of achieving its multiple functions such as anti-icer, a carburetor anti-foulant, and a corrosion inhibitor. In general, one employs at least about 5 p.p.m. such as about 5 to 500 p.p.m., for example from about 10 to 100 p.p.m., but preferably about 25 to 75 p.p.m. In practice, from economic considerations, the least amount

of additive capable of effecting the desired results is employed.

The product prepared in Example 1 was evaluated according to the following tests.

It is to be noted that the solution of the additive employed was 75% active.

## TEST I.—CARBURETOR ICING EVALUATION

Test conditions: 40° F. intake air; 90%  $\pm$  5% humidity; continuous air circulation.

Test procedure:

- (1) Start cold engine.
- (2) Accelerate to 1500 r.p.m. and maintain for one minute.
- (3) Decelerate to idle r.p.m. and idle engine for one-half minute. Observe and record engine stalling characteristics.
- (4) If engine stalls, immediately restart and rerun the cycles described by item (1) through (3) above.

## TEST RESULTS

| Fuel Sample                                    | Number of Stalls | Total Test Cycles | Percent Reduction in Stalls |
|------------------------------------------------|------------------|-------------------|-----------------------------|
| Base Gasoline                                  | 12               | 17                |                             |
| Additive Example 1 (75% octane)<br>(50 p.p.m.) | 7                | 13                | 24                          |

## TEST II.—DYNAMIC RUST TEST FOR PETROLEUM FUELS

Apparatus: As specified in ASTM method D665-60

Procedure:

- (1) Insert polished spindle into 300 ml. of test fuel.
- (2) Allow spindle 10 minutes static and 20 minutes dynamic wetting time.

- (3) Add 30 ml. of distilled water and stir for 4 hours.  
 (4) Remove spindle, wash with isopropyl alcohol, then isoctane, air dry and grade immediately.

## RATING

| Appearance of Spindle    | Rating               | Designation |
|--------------------------|----------------------|-------------|
| Free of rust.....        | Passes.....          | R-1         |
| Few spots.....           | do.....              | R-2         |
| Less than 5% rusted..... | Borderline pass..... | R-3         |
| 5% to 50% rusted.....    | Does not pass.....   | R-4         |

## RESULTS: TEST FUEL—PREMIUM GASOLINE

| Additive                             | Concen-<br>tration,<br>p.p.m. | Rating |
|--------------------------------------|-------------------------------|--------|
| None.....                            | .....                         | R-4    |
| Additive Example 1 (75% octane)..... | 15                            | R-2    |
| Do.....                              | 25                            | R-1    |

## TEST III.—STATIC RUST TEST FOR PETROLEUM FUELS

## Procedure:

- (1) Presoak a polished spindle (spindle prepared as prescribed in ASTM Method D665-60) for 15 minutes in 300 ml. of the fuel sample in a pint container.
- (2) Remove spindle and add 3 ml. of distilled water.
- (3) Hand shake vigorously for 30 seconds, then replace spindle immediately.
- (4) Take daily readings for 6 days.
- (5) Rate by standard spindle method; R-1 to R-4. With readings of R-4 and higher, an estimate of the percent of rusted area should be made to the nearest 10 percent.

## RESULTS: TEST FUEL—PREMIUM GASOLINE

| Additive                             | Concen-<br>tration,<br>p.p.m. | Rating in degrees |     |     |     |     |     |
|--------------------------------------|-------------------------------|-------------------|-----|-----|-----|-----|-----|
|                                      |                               | 1                 | 2   | 3   | 4   | 5   | 6   |
| None.....                            | .....                         | R-3               | R-3 | R-3 | R-3 | R-3 | R-9 |
| Additive Example 1 (75% octane)..... | 25                            | R-1               | R-1 | R-1 | R-1 | R-1 | R-1 |

## TEST IV.—EVALUATION OF GASOLINE ADDITIVE TIME FOR CARBURETOR DETERGENCY EFFECTIVENESS

Equipment—1954 Model 6 cylinder Plymouth engine. Displacement 217.8 cubic inch.

The metallic throttle body section of the carburetor is replaced by a specially machined clear plastic throttle body. This section contains all of the fuel and air passages including the adjustments as well as the butterfly valve.

During the "dirty-up" sequence of the evaluation, the engine is operated with the full crankcase blowby returned to the carburetor inlet. An air cleaner is also used during this sequence. A base fuel containing no detergent is used. The duration of "dirty-up" time is controlled by the percentage of area where deposits adhere to the throttle body throat through visual observation. When deposits appear to be at the desired level the engine is shut down. The throttle body is removed and rated for deposits. Rating is accomplished by means of inserting a thin cylindrical plastic template into the throttle body throat. The template has 100 equally divided spaces. Coverage by deposit of one space is 1% area. The deposits are classified as black (opaque) and light black (translucent).

For the "clean-up" sequence the blowby is not returned to the carburetor inlet. The throttle body is installed with the deposits intact. The engine is operated for five hours under identical conditions without changing any settings. The same base fuel is used containing the detergent added according to instructions. At the end of five hours the throttle body is again removed for rating of the deposits.

The throttle control is by means of an automatic control which suddenly accelerates from low idle (400 r.p.m.) to high idle (1500 r.p.m.) for an instant (approximately one second) then decelerates to the norm. This action occurs six times in rapid succession at eight minute intervals during the fuel evaluation.

Appropriate instrumentation is provided to insure uniformity of engine conditions. The crankcase blowby is also measured before and after the evaluation to establish that the test severity does not change from one run to the next.

A premium grade base fuel is used for reference runs and the additive is added to this same fuel for evaluation.

- 15 The rating method is normally reported by the percentage of the black deposit "clean-up" and the light black deposit "clean-up."

## EVALUATION OF GASOLINE ADDITIVE FOR CARBURETOR DETERGENCY EFFECTIVENESS—STANDARD TWO SEQUENCE TEST

|    |                                                | Black                | Light                         | Total          |
|----|------------------------------------------------|----------------------|-------------------------------|----------------|
|    |                                                | Clean-up,<br>percent | Black<br>Clean-up,<br>percent |                |
| 25 | Additive Example, 150 p.p.m. (75% octane)..... | 24<br>30<br>4        | -2<br>-4<br>6                 | 22<br>26<br>10 |
|    | Average.....                                   | 19                   | 0                             | 19             |

- 30 The above additive is particularly effective in removing the Black Clean-up which represents the denser black deposits. In this respect it is superior to an equal amount of a commercial additive—acylated oleic acid



reaction product.

## TEST V.—WATER TOLERANCE TEST

## Procedure:

- 40 (1) Add 80 cc. of inhibited isoctane and 20 cc. of distilled water to a 100 cc. graduate.
- (2) Hand shake 200 times.
- (3) Allow to settle for five minutes.
- (4) Observe interface and emulsion that occur in either phase.

50 The additive of Example 1 (75% octane), 30 p.p.m., yielded a clear, one phase system. In contrast a commercial additive, 30 p.p.m., formed by acylating



55 with oleic acid yielded a two phase system, i.e. the lower layer of which was cloudy.

Solutions of the additive of Example 1 have improved low temperature handling properties (pour point—50° F.) as compared to a commercial additive formed from reacting oleic acid with



60 in the same solvent concentration. This affords an important commercial advantage during the winter season.

65 Salts of the acylated polyamines may be salts of organic or inorganic acids such as mineral acids-HCl, sulfuric acid, phosphoric, etc. and naphthenic acid, acetic acid, dimeric acids, maleic acids, phthalic acids, benzoic acid, etc., i.e. aliphatic, arylic, saturated, unsaturated, monocarboxylic, polycarboxylic, etc. acids and mixtures thereof.

70 Having thus described my invention what I claim as new and desire to obtain by Letters Patent is:

- 75 1. A hydrocarbon motor fuel of the gasoline boiling range characterized by the presence of a composition, in an amount capable of achieving multiple anti-icing, anti-fouling and corrosion inhibiting functions, said composi-

9

tion being a mixture of predominantly an imidazoline of the formula



with a small amount of an amide of the formula



wherein R is naphthyl derived from naphthenic acid having a molecular weight of about 200 to 500, said mixture being prepared by reacting one mole of said naphthenic acid and one mole of aminoethylethanolamine at 170° C.

## References Cited

UNITED STATES PATENTS

|    |           |         |                  |    |    |    |
|----|-----------|---------|------------------|----|----|----|
|    | 2,773,879 | 12/1956 | Sterlin          | 44 | 63 | XR |
|    | 2,839,371 | 6/1958  | Sigworth et al.  | 44 | 63 |    |
| 5  | 2,839,372 | 6/1958  | Lindstrom et al. | 44 | 71 | XR |
|    | 3,014,792 | 12/1961 | Capowski et al.  | 44 | 63 |    |
|    | 3,033,664 | 5/1962  | Pethrick et al.  | 44 | 63 |    |
|    | 3,305,329 | 2/1967  | Sims et al.      | 44 | 63 |    |
| 10 | 3,337,472 | 8/1967  | Littler et al.   | 44 | 66 | XR |
|    | 2,622,018 | 12/1952 | White et al.     | 44 | 63 |    |
|    | 3,036,902 | 5/1962  | Hamer et al.     | 44 | 63 | X  |

DANIEL E. WYMAN, Primary Examiner

W. J. SHINE, Assistant Examiner

U.S. Cl. X.R.

44—71; 252—392